

United States Patent [19]  
Webster



US005320803A

[11] Patent Number: 5,320,803  
[45] Date of Patent: \* Jun. 14, 1994

[54] PROCESS FOR MAKING  
ALUMINUM-LITHIUM ALLOYS OF HIGH  
TOUGHNESS

[75] Inventor: Donald Webster, Saratoga, Calif.

[73] Assignee: Comalco Aluminium Limited,  
Melbourne, Australia

[\*] Notice: The portion of the term of this patent  
subsequent to Feb. 4, 2009 has been  
disclaimed.

[21] Appl. No.: 771,907

[22] Filed: Oct. 4, 1991

Related U.S. Application Data

[63] Continuation-in-part of Ser. No. 328,364, Mar. 24,  
1989, Pat. No. 5,085,830.

[51] Int. Cl. 5 ..... C22C 1/02

[52] U.S. Cl. ..... 420/528; 75/678;

75/686; 420/533; 420/543

[58] Field of Search ..... 420/402, 407-410,  
420/528, 529, 531-535, 537, 540-546, 549, 552,  
553; 148/406, 415-417, 420, 437-440; 75/678,  
686

[56] References Cited

U.S. PATENT DOCUMENTS

4,049,248 9/1977 Gjosteen et al. ..... 266/202  
4,735,774 4/1988 Narayanan et al. ..... 420/533  
5,032,359 7/1991 Pickens et al. ..... 420/533  
5,085,830 2/1992 Webster ..... 420/528

FOREIGN PATENT DOCUMENTS

130985 7/1946 Australia ..... 420/402

OTHER PUBLICATIONS

Frost, P. D., Jackson, J. H., Loonam, A. C., and Lorig,

C. H. "The Effect of Sodium Contamination on Mag-  
nesium-Lithium Base Alloys," *Transactions AIME, Journal of Metals*, vol. 188, pp. 1171-1172, Sep. 1950.

Webster, "The Effect of Low Melting Point Impurities on the Properties of Aluminum-Lithium Alloys," *Metallurgical Transactions A*, vol. 18A, pp. 2181-2193, Dec. 1987.

Kojima et al., "Microstructural Characterization and Mechanical Properties of a Spray-Cast Al-Li-Cu-Mg-Zr Alloy," *Proceeding of the 5th International Aluminum-Lithium Conference*, Williamsburg, pp. 85-91 (Mar. 27-31, 1989).

Fager et al., "A Preliminary Report on Cleavage Fracture in Al-Li Alloys," *Scripta Metallurgica*, vol. 20, pp. 1159-1164 (1986).

Miller et al., "Sodium Induced Cleavage Fracture in High Strength Aluminum Alloys," *Scripta Metallurgica*, vol. 21, pp. 663-668 (1987).

Metals Handbook, vol. 15 Casting, 9th ed. pp. 84-85, 460-463, 746-749.

Hownmet, TSIR # 1781 (dated Mar. 17, 1987).

Primary Examiner—Melvyn J. Andrews

Assistant Examiner—Robert R. Koehler

Attorney, Agent, or Firm—Nikaido, Marmelstein,  
Murray & Oram

[57] ABSTRACT

The toughness of Al-Li, Al-Mg and Mg-Li alloys is increased by a melting and refining process designed to reduce the concentration of alkali metal impurities below specified levels. The hydrogen and chlorine gas constituents are also significantly reduced.

10 Claims, 16 Drawing Sheets





FIG.1



FIG.2



FIG.3



FIG.4



FIG. 5



FIG.6



FIG. 7



FIG.8



FIG.10



FIG.9





FIG.13



FIG.14



FIG.15



FIG.16



**FIG.17**



FIG.18



FIG.20



FIG.19



FIG.21



FIG.22



FIG.23



FIG.24



FIG.25



FIG.26

## PROCESS FOR MAKING ALUMINUM-LITHIUM ALLOYS OF HIGH TOUGHNESS

This application is a continuation-in-part of U.S. application Ser. No. 328,364, filed Mar. 24, 1989 now U.S. Pat. No. 5,085,830.

### FIELD OF THE INVENTION

This invention relates to improving the physical properties of alloys that form liquid grain boundary phases at ambient temperatures due to alkali metal impurities such as Al-Li, Al-Mg, and Mg-Li metallic products and more particularly to methods for increasing the toughness, corrosion cracking resistance and ductility of such products without loss of strength.

### BACKGROUND OF THE INVENTION

High strength aluminum alloys and composites are required in certain applications, notably the aircraft industry where combinations of high strength, high stiffness and low density are particularly important. High strength is generally achieved in aluminum alloys by combinations of copper, zinc and magnesium. High stiffness is generally achieved by metal matrix composites such as those formed by the addition of silicon carbide particles or whiskers to an aluminum matrix. Recently Al-Li alloys containing 2.0 to 2.8% Li have been developed. These alloys possess a lower density and a higher elastic modulus than conventional non-lithium containing alloys.

The preparation and properties of aluminum based alloys containing lithium are widely disclosed, notably in J. Stone & Company, British patent No. 787,665 (Dec. 11, 1957); Ger. Offen. 2,305,248 (National Research Institute for Metals, Tokyo, Jan. 24, 1974); Racicot, U.S. Pat. No. 3,343,948 (Sep. 26, 1967); and Peel et al., British Patent No. 2,115,836 (Sep. 14, 1983).

Unfortunately, high strength aluminum-lithium alloys are usually characterized by low toughness, as evidenced by impact tests on notched specimens (e.g., Charpy tests, See: Metals Handbook, 9th Ed. Vol. 1, pages 689-691) and by fracture toughness tests on fatigue precracked specimens where critical stress intensity factors are determined.

There have been two basic techniques used to improve the toughness of Al-Li alloys.

1. Techniques commonly used for other aluminum alloys, such as alloying (Cu, Zn, Mg), stretching 1 to 5% before aging to refine precipitation, control of recrystallization and grain growth with Zr (0.1%) and the control of initial grain size by the use of powder metallurgy.

2. The production of dispersoids in amounts greater than needed for recrystallization control using 0.5 to 2% of Mn, Zr, Fe, Ti and Co to homogenize slip distribution.

In the last 10 years these methods have had some success but the toughness of Al-Li alloys still falls short of that of conventional aluminum alloys.

Conventional techniques, for improving the toughness of Al-Li alloys, have not included the use of a vacuum melting and refining treatment. Aluminum alloys are typically melted in air; although, vacuum melting is used by some manufacturers of high quality aluminum investment castings, such as Howmet Turbine Components Corporation who make castings of A357 and A201, to avoid dross formation. (Bouse, G. K.

and Behrendt, M. R. "Advanced Casting Technology Conference", edited by Easwaren, published by ASM, 1987).

5 Howmet has also made experimental Al-Li-Cu-Mg investment castings by vacuum melting (Proceedings of the Al-Li Alloys Conference, held in Los Angeles March, 1987, pp. 453-465, published by ASM International) to reduce reactions between lithium and air and to reduce hydrogen pick up which occurs when lithium reacts with moisture in the air. Commercial Al-Li alloys are usually melted under an argon atmosphere which accomplishes these objectives less efficiently than vacuum but is an improvement over air melting.

10 Al-Li alloys although having many desirable properties for structural applications such as lower density, increased stiffness and slower fatigue crack growth rate compared to conventional aluminum alloys are generally found to have the drawback of lower toughness at equivalent strength levels.

15 Conventional high strength Al-Li alloys have resistance to stress-corrosion cracking in the short transverse (S-T) direction less than about 200 MPa (29 ksi) in the peak aged to overaged condition, e.g., alloy 7075 has a threshold stress for stress corrosion cracking in the S-T direction in the range of about 300 MPa (42 ksi) in the T73 condition to about 55 MPa (8 ksi) in the T6 condition.

20 25 30 35 The magnesium-lithium family of alloys when manufactured by conventional techniques are known to suffer from stress corrosion cracking, overaging, instability and creep at low temperatures. Razim, et al., Advanced Materials & Processes, Vol. 137, Issue 5, pp. 43-47 (May, 1990). Some of the problems in Mg-Li alloys have been associated with alkali metal impurities and it has been observed that Na levels above 20 ppm reduced room temperature ductility. Payne et al., JIM, Vol. 86, pp. 351-352 (1957-58). Some Mg-Li alloy specifications set the Na limit to less than 20 ppm for wrought products and 10 ppm for castings.

### ADVANTAGES AND SUMMARY OF THE INVENTION

40 45 50 Advantages of the subject invention are that it provides a simple, versatile and inexpensive process for improving the toughness of Al-Li, Al-Mg and Mg-Al alloys that is effective on both virgin and scrap source alloys. The invention also provides alloys with heretofore unattainable combinations of properties especially toughness, corrosion cracking resistance and ductility without loss of strength.

55 Another advantage of the subject invention is that it avoids formation and incorporation of various metal oxides and other impurities known to cause embrittlement and commonly associated with, e.g., powder metallurgy techniques, that involve heating and/or spraying the product alloy in air or other gases.

60 65 It has now been discovered that improved combinations of high strength, high toughness and good ductility can be obtained in aluminum alloys containing primary alloying elements selected from the group consisting of Li and Mg by processing the alloys in the molten state under conditions that reduce alkali metal impurities (AMI), i.e., (Na, K, Cs, Rb) content. Preferably the process also reduces gas impurities such as hydrogen and chlorine and reduces the formation of detrimental oxides. The processing technique involves subjecting the molten alloy to conditions that remove alkali metal impurity, e.g., a reduced pressure for a sufficient time to

reduce the aggregate concentration alkali metal impurities to less than about 5 ppm, preferably, less than about 3 ppm and more preferably less than 1 ppm. Generally, the best observed results occurred at less than 0.8 and 0.5 ppm. It has also been found that the presence of certain combinations of alkali metal impurities in relative proportions which form low melting point eutectic mixtures requires removal of alkali metal impurities to levels below the higher level, e.g., 5 ppm, mentioned above to achieve the property improvement provided by this invention. It is believed that this is because the eutectic mixtures remain liquid and they cause embrittlement at temperatures well below room temperature. Certain combinations of Na, K and Cs are known to remain liquid down to minus 78° C.

As noted above the process also beneficially reduces the gas (hydrogen and chlorine) content of the alloys which is expected to provide an additional, improvement in quality by reducing the formation of surface blisters and giving superior environmentally related properties such as stress corrosion resistance. Preferably, the hydrogen concentration is reduced to less than about 0.2 ppm and more preferably, less than about 0.1 ppm. Preferably the chlorine concentration is reduced to less than about 1.0 ppm and more preferably less than about 0.5 ppm.

The alloys of this invention may be used to make high strength composite materials by dispersing particles such as fibers or whiskers of silicon carbide, graphite, carbon, aluminum oxide or boron carbide therein. The term aluminum based metallic product is sometimes used herein to refer generally to both the alloys and alloy composites of the invention.

The present invention also provides improved Mg-Li alloys, for example, the experimental alloy LA141A, comprising magnesium base metal, lithium primary alloying element and less than about 1 ppm, preferably less than about 0.1 ppm, and most preferably less than about 0.01 ppm of each alkali metal impurity selected from the group consisting of sodium, potassium, rubidium and cesium. Generally, the alkali metal impurity concentrations in Mg-Li alloys should be less than 10 ppm Na, less than 5 ppm K and less than 1.5 ppm Cs and Rb. As with the Al-Li and Al-Mg alloys described above the hydrogen concentration is preferably less than about 0.2 ppm, more preferably less than about 0.1 ppm and the chlorine concentration is preferably less than about 1.0 ppm, and more preferably less than about 0.5 ppm.

The Mg-Li alloys typically include about 13.0 to 15.0 percent lithium and about 1.0 to 1.5% aluminum, preferably about 14.0% lithium, and about 1.25% aluminum. The Mg-Li of this invention can be made by the processes described herein in connection with the Al-Li and Al-Mg alloys.

#### BRIEF DESCRIPTION OF THE DRAWINGS

FIG. 1 is a plot of 0.2% tensile yield strength versus the Charpy impact energy at each strength level from a commercially produced A12090 alloy and a vacuum refined A12090 alloy produced by the process described herein. Property measurements are taken from both the center one third of the extrusion and the outer one third of each extrusion.

FIG. 2 is a plot of the 0.2% tensile yield strength versus the Charpy impact energy at each strength level for alloy 2 described in Example 2 and produced by the vacuum refining process described herein.

FIG. 3 is a plot of the 0.2% tensile yield strength versus the Charpy impact energy at each strength level for alloy 3 described in Example 3 and produced by the vacuum refining process described herein.

FIG. 4 is a plot of the 0.2% tensile yield strength versus the Charpy impact energy at each strength level for alloy 4 described in Example 4 and produced by the vacuum refining process described herein.

FIG. 5 is a plot of the 0.2% tensile yield strength versus the Charpy impact energy at each strength level for three alloys containing 3.3% Li and other alloying elements. Alloys 5 and 6 described in Example 5 were produced by the vacuum refining process described herein while alloy 1614 was produced by a powder metallurgy process and described in U.S. Pat. No. 4,597,792 and Met. Trans. A, Vol. 19A, March 1986, pp 603-615.

FIG. 6 is a plot of the concentration of H, Cl, Rb and Cs versus refining time for alloys 1 to 6.

FIG. 7 is a plot of Na and K concentration versus refining time for alloys 1, 3, 4 and 5.

FIG. 8 is a plot comparing the stress corrosion resistance of alloys 1, 3 and 4 of the invention to conventional Al-Li alloys.

FIG. 9 is a plot of Total Crack Length vs. Augmented Strain from Table II.

FIG. 10 is a plot of Total Crack Length vs. Augmented Strain from Table III.

FIGS. 11 to 14 are plots of % yield strength v. elongation of % for several 2090 and 8090 type Al-Li alloys having various alkali metal impurity levels for alloys 1(2090), 2(8090) and E to P.

FIG. 15 and 16 are plots of 0.2% yield strength versus alkali metal impurity Na+4 K for test alloys 1(2090), 2(8090) and E to P.

FIGS. 17 and 18 are plots of elongation % versus alkali metal impurity (Na+4 k) for test alloys 1(2090), 2(8090) and E to P.

FIGS. 19 to 22 are plots of Charpy impact valves versus alkali metal impurity (Na+4 K).

FIG. 23 is a plot of a calculated loss in toughness versus total alkali metal impurity.

FIG. 24 is a plot of the mechanical properties modified 5083 alloys A,B and C.

FIGS. 25 and 26 are plots of the mechanical properties of Mg-Li alloys X, Y and Z.

#### DETAILED DESCRIPTION OF THE INVENTION

The present invention is applicable to aluminum based metallic materials containing lithium or magnesium as a primary alloying element and magnesium base of metallic materials including lithium, including both alloys and composites. The term 'primary alloying element' as used herein means lithium or magnesium in amounts no less than about 0.5%, preferably no less 1.0% by weight of the alloy. These materials can have a wide range of composition and can contain in addition to lithium or magnesium any or all of the following elements: copper, magnesium or zinc as primary alloying elements. All percents (%) used herein mean weight % unless otherwise stated.

Examples of high strength composites to which the present invention is also applicable include a wide range of products wherein Al-Li, Al-Mg and Mg-Li matrices are reinforced with particles, such as whiskers or fibers, of various materials having a high strength or modulus. Examples of such reinforcing phases include boron

fibers, whiskers and particles; silicon carbide whiskers and particles, carbon and graphite whiskers and particles and, aluminum oxide whiskers and particles.

Examples of metal matrix composites to which the present invention is applicable also include those made by ingot metallurgy where lithium and magnesium are important alloying elements added for any or all of the following benefits, lower density, higher stiffness or improved bonding between the matrix and the ceramic reinforcement or improved weldability. The benefits conferred by the present invention on Al-Li, Al-Mg and Mg-Li composite materials are similar to those conferred to the corresponding alloys themselves, particularly, a combination of improved properties including higher toughness and ductility. Modern commercial Al-Li and Al-Mg alloys generally have a total (AMI) content of less than about 10 ppm which is introduced as impurity in the raw materials used for making the alloys. Mg-Li alloys also have high AMI contents corresponding to the larger proportions of lithium used therein.

Typically, a major portion of AMI contamination comes from the lithium metal which often contains about 50 to 100 ppm of both sodium and potassium. Since Al-Li alloys usually contain about 2 to 2.8% Li the amount of sodium or potassium contributed by the lithium metal is usually in the range about 1 to 2.8 ppm. Additional AMI can be introduced through chemical attack by the Al-Li on the refractories used in the melting and casting processes. Therefore a total AMI content of about 5 ppm would not be unusual in commercial Al-Li ingots and mill products.

Alkali metal impurity exist in Al-Li alloys as grain boundary liquid phases (Webster, D. met. Trans. A, Vol. 18A, December 1987, pp. 2181-2193.) which are liquid at room temperature and can exist as liquids to at least the ternary eutectic of the Na-K-Cs system at 195° K. (-78° C.). These liquid phases promote grain boundary fracture and reduce toughness. An estimate of the loss of toughness can be obtained by testing at 195° K. or below where all the liquid phases present at room temperature have solidified. When this is done the toughness as measured by a notched Charpy impact test has been found to increase by up to four times.

The present invention exploits the fact that all the AMI have higher vapor pressures and lower boiling points than either aluminum, lithium, magnesium or the common alloying elements such as Cu, Zn, Zr, Cr, Mn and Si. This means that the AMI will be removed preferentially from alloys including these and similar elements when the alloys are maintained in the molten state under reduced pressure for a sufficient time. The first impurities to evaporate will be Rb and Cs followed by K with Na being the last to be removed. The rate of removal of the AMI from the molten Al-Li bath will depend on several factors including the pressure in the chamber, the initial impurity content, the surface area to volume ratio of the molten aluminum and the degree of stirring induced in the molten metal by the induction heating system.

In a preferred embodiment, an increase in the AMI evaporation rate may be obtained by purging the melt with an inert gas such as argon introduced into the bottom of the crucible through a refractory metal (Ti, Mo, Ta) or ceramic lance. The increase in removal rate due to the lance will depend on its design and can be expected to be higher as the bubble size is reduced and the gas flow rate is increased. The theoretical kinetics of

the refining operation described above can be calculated for a given melting and refining situation using the principles of physical chemistry as for example those summarized in the Metals Handbook Vol. 15, Casting, published in 1988 by ASM International.

The refining process is preferably carried out in a vacuum induction melting furnace to obtain maximum melt purity. However, in order to incorporate this technique into commercial Al-Li, Al-Mg and Mg-Li alloy production practice, the refining operation can take place in any container placed between the initial melting furnace/crucible and the casting unit, in which molten alloys can be maintained at the required temperature under reduced pressure for a sufficient time to reduce the AMI to a level at which their influence on mechanical properties particularly toughness is significantly reduced.

The process of the present invention may be operated at any elevated temperature sufficient to melt the aluminum base metal and all of the alloying elements, but should not exceed the temperature at which desired alloy elements are boiled-off. Useful refining temperatures are in the range of about 50° to 200° C., preferably about 100° C., above the melting point of the alloy being refined. The optimum refining temperature will vary with the pressure (vacuum), size of the melt and other process variables.

The processing pressure (vacuum) employed in the process to reduce the AMI concentration to about 1 ppm or less, i.e., refining pressure, is also dependent upon process variables including the size of the melt and furnace, agitation, etc. A useful refining pressure for the equipment used in the Examples hereof was less than about 200  $\mu\text{m}$  Hg.

The processing times, i.e., the period of time the melt is kept at refining temperatures, employed in the process to reduce the AMI concentration to about 1 ppm or less are dependent upon a variety of factors including the size of the furnace, and melt, melt temperature, agitation and the like. It should be understood that agitation with an inert gas as disclosed herein will significantly reduce processing times. Useful processing times for the equipment used in the Examples herein ranged from about 40 to 100 minutes.

It should be understood that the temperature, time and pressure variables for a given process are dependent upon one another to some extent, e.g., lower pressures or longer processing times may enable lower temperatures. Optimum time, temperature and pressure for a given process can be determined empirically.

The following examples are offered for purposes of illustration and are not intended to either define or limit the invention in any manner.

#### EXAMPLE 1

An A12090 alloy made by standard commercial practice was vacuum induction melted and brought to a temperature of about 768° C. under a reduced pressure of about 200  $\mu\text{m}$  Hg. A titanium tube with small holes drilled in the bottom four inches of the tube was inserted into the lower portion of the molten metal bath and argon gas passed through the tube for five minutes. The gas was released well below the surface of the melt and then bubbled to the surface. The melt was then given a further refining period of about fifty minutes using only the reduced pressure of the vacuum chamber to reduce the AMI. The melt was grain refined and cast using standard procedures.

Five inch diameter billets were extruded into a flat bar 1.77 inches by 0.612 inches thick. The composition of the original melt and the vacuum remelted material are given in Table 1.

TABLE I

| CHEMICAL ANALYSES OF MATERIAL BEFORE AND AFTER VACUUM REFINING |        |                   |                       |                   |
|----------------------------------------------------------------|--------|-------------------|-----------------------|-------------------|
| ELEM-<br>MENT                                                  | A12090 | VACUUM<br>REFINED | ANALYSIS<br>TECHNIQUE | ANALYSIS<br>UNITS |
| Li                                                             | 1.98   | 1.96              | ICP                   | Wt. Pct.          |
| Cu                                                             | 2.3    | 2.4               | ICP                   | Wt. Pct.          |
| Zr                                                             | 0.13   | 0.13              | ICP                   | Wt. Pct.          |
| Na                                                             | 3.2    | N.D.              | ES                    | PPM               |
| Na                                                             | 3.1    | 0.480             | GDMS                  | PPM               |
| Na                                                             | 0.480* | SIMS              | PPM                   | PPM               |
| K                                                              | 0.600  | 0.050             | GDMS                  | PPM               |
| K                                                              | 0.008  | SIMS              | PPM                   | PPM               |
| Cs                                                             | <0.008 | <0.008            | GDMS                  | PPM               |
| Cs                                                             | 0.015  | SIMS              | PPM                   | PPM               |
| Rb                                                             | 0.042  | <0.013            | GDMS                  | PPM               |
| Rb                                                             | .0005  | SIMS              | PPM                   | PPM               |
| Cl                                                             | 3.5    | 0.500             | GDMS                  | PPM               |
| H (bulk)                                                       | 1.0    | 0.140             | LECO                  | PPM               |

\*SIMS analyses were standardized using GDMS and ES results.

PPM = parts per million

GDMS = glow discharge mass spectrometry

SIMS = secondary ion mass spectrometry

ES = emission spectrometry

LECO = hydrogen analysis by LECO Corporation, 3000 Lakeview Ave. St. Joseph, Mi, 49085 USA - melting alloy under a stream of nitrogen gas and determining the hydrogen content by change in thermal conductivity.

= not determined

It can be seen that the desirable alloying element concentrations, i.e., Li, Cu and Zr, were substantially unchanged during the vacuum melting and refining process, but the undesirable impurities, Na, K, Rb, H and Cl were markedly reduced. Since Cs was already below the detection limit of GDMS before the refining process began, no change in this element could be detected.

The Charpy impact toughness values of specimens produced from flat bar extrusions of the vacuum refined A12090 and specimens produced from a commercial A12090 alloy are compared as a function of 0.2% yield strength in FIG. 1. The strength-toughness combinations for the vacuum refined alloy surpass those of the commercial alloy at all strength levels and also exceeds these property combinations of the usually superior conventional alloys, A17075 and A12024 (not shown).

The strength-toughness combinations of the extrusion edges are superior to those of the extrusion centers for this alloy and for the other alloys described in the examples below. This difference in properties occurs in extrusions of both Al-Li and conventional aluminum alloys and is related to a change in 'texture' across the extrusion width. Texture in this case is meant to include grain size and shape, degree of recrystallization and preferred crystallographic orientation. The texture for the new Al-Li alloys is more pronounced than in commercial Al-Li alloys and conventional aluminum alloys. The degree of texture can be controlled by extrusion temperature, extrusion ratio and extrusion die shape.

#### EXAMPLE 2

An alloy containing 1.8% Li, 1.14% Cu, 0.76% Mg and 0.08% Zr, was given a vacuum refining treatment similar to that in Example 1 except that an argon lance was not used. It was then cast and extruded to flat bar and heat treated in the same manner as described in Example 1. The toughness properties (FIG. 2) again greatly exceed those of commercial Al-Li alloys at all

strength levels. In many cases the toughness exceeds 100 ft. lbs. and is higher than that for most steels.

#### EXAMPLE 3

5 An alloy containing 2.02% Li, 1.78% Mg, and 0.08% Zr was given a vacuum refining treatment similar to that described in Example 2. It was then extruded and heat treated and its strength and toughness were evaluated and are illustrated in FIG. 3. This specimen was so tough that it could not be broken on the 128 ft. lb. Charpy testing machine capable of breaking specimens from almost all steel alloys.

#### EXAMPLE 4

15 An alloy containing 2.4% Li, 0.88% Mg, 0.33% Cu and 0.18% Cr was given a vacuum refining treatment similar to that in Example 2. It was then extruded and heat treated and its strength and toughness were evaluated as in previous Examples and illustrated in FIG. 4. 20 Again strength-toughness combinations greatly superior to those of conventional alloys were obtained.

#### EXAMPLE 5

25 Two alloys (alloys 5 and 6) containing a higher than normal Li level (3.3% by weight) to obtain a very low density (0.088 lb/cu. in.) were given a vacuum refining treatment similar to that described in Example 2. The alloys were then cast, extruded and heat treated as in the previous examples. The strength-toughness combinations were evaluated and are shown in FIG. 5.

30 The high lithium level reduces the toughness compared to the alloys in Examples 1 to 4 but the properties are generally comparable to those of commercial Al-Li alloys and are superior to those of the much more expensive powder metallurgy alloys (U.S. Pat. No. 4,597,792 issued 1986 to Webster, D.) with the same lithium content as illustrated in FIG. 5. The compositions of the vacuum refined alloys described this example are:

40 Alloy 5 . . . 3.3% Li, 1.1% Mg, 0.08% Zr  
Alloy 6 . . . 3.3% Li, 0.56% Mg, 0.23% Cu, 0.19% Cr  
Alloy 7 . . . 2.9% Li, 1.02% Mg, 0.41% Cu, 0.1 Zr, 0.010 Fe, 0.12 Si, and 4 ppm Na (not described).

#### EXAMPLE 6

45 The above-described alloys 1 to 6 were analyzed for AMI concentration after refining steps of varying duration. The results of those analyses are summarized in Table II below and illustrated in FIGS. 6 and 7. It should be noted that the inert gas lance described above was only used for refining alloy 1, Example 1 which had the lowest final K and Na concentrations.

TABLE II  
CHEMICAL COMPOSITION  
AS A FUNCTION OF REFINING TIME

| ALLOY                 | IMPURITY CONCENTRATION (PPB) |      |     |    |      |      | REFINING<br>TIME<br>(Minutes) |
|-----------------------|------------------------------|------|-----|----|------|------|-------------------------------|
|                       | Na                           | K    | Rb  | Cs | H    | Cl   |                               |
| 1- start <sup>1</sup> | 3100                         | 600  | 42  | <8 | 1000 | 3500 | 55                            |
|                       | 480                          | 50   | <13 | <8 | 140  | 500  |                               |
| 2- start              |                              |      |     |    | 1350 |      | 68                            |
|                       |                              |      |     |    | 120  |      |                               |
| 3- start              | 2000                         | 1000 | 60  | 5  | 1420 |      | 104                           |
|                       | 545                          | 325  | <8  | <6 | 70   | 1044 |                               |
| 4- start              | 2200                         | 1200 | 72  | 6  | 1700 |      | 53                            |
|                       | 602                          | 206  | <8  | <6 | 300  | 1540 |                               |
| 5- start              | 2650                         | 1650 | 100 | 8  | 2300 |      | 48                            |
|                       | 645                          | 341  | <9  | <6 | 540  | 755  |                               |

TABLE II-continued

| ALLOY    | CHEMICAL COMPOSITION AS A FUNCTION OF REFINING TIME |   |    |    |      | REFINING TIME (Minutes) |
|----------|-----------------------------------------------------|---|----|----|------|-------------------------|
|          | Na                                                  | K | Rb | Cs | H    |                         |
| 6- start |                                                     |   |    |    | 3500 |                         |
| finish   |                                                     |   |    |    | 420  | 46                      |

<sup>1</sup>The start values are based on data published in Webster, D. Met. Trans. A, Vol. 18A, Dec. 1987 pp 2181-2183.

Based on the above data it is estimated that a minimum refining time of about 100 minutes is required to reduce the AMI to their equilibrium values (lowest attainable value). Although this estimate applies only to the melt used, i.e., about 100 lbs. in a 10 inch diameter by 14 inch deep crucible it illustrates how the effectiveness of the invention can be estimated.

#### EXAMPLE 7—Stress Corrosion Cracking Resistance

Stress corrosion tests were performed on extruded lengths of the Al-Li alloys 1, 3 and 4, described in the preceding Examples. The purpose of the tests was to determine the threshold stress of stress corrosion cracking for each alloy in the S-T direction.

Ten turning fork samples of each Alloy (Alloys 1, 3, and 4) were machined from the center of the extrusions with a flat testing surface normal to the extrusion axis.

The specimens were loaded by deflecting the legs of the fork to predetermined stress levels between about 100 Mpa (i.e., 15 ksi) and 450 (i.e., 65 ksi) and subjected to alternate immersion testing in 3.5% NaCl solution in accordance with ASTM G44.

None of the specimens fractured during the 28 day testing period regardless of the stress used.

Alloy 1 suffered general corrosion with numerous pits and initial examination of the pits indicated the possible presence of short cracks. Higher magnification metallographic examinations showed one stress corrosion crack on a sample tested at 380 MPa (i.e., 55 ksi) which had propagated about 80% through the section.

Alloy 3 suffered no general corrosion and had its surface remained conditions almost unchanged from the pretest conditions. Alloy 4 suffered no general corrosion and was only slightly stained on the surface.

Only Alloy 1 showed a threshold; alloys 3 and 4 showed no failures at any of the test stress levels.

The stress corrosion cracking threshold stress for conventional alloys 7075 and 2024 are shown in FIG. 8.

#### EXAMPLE 8—WELDABILITY

The weldability of Alloys 1 to 5 of the invention was evaluated by a Varestraint test using augmented strains of up to 4%. The test subjected the weld pool to controlled amounts of strain during welding. The total crack length and maximum crack length were measured and plotted against augmented strain in FIG. 9 to obtain comparative weldabilities for the different Alloys.

The Varestraint tests were performed using a gas tungsten arc welding technique with constant welding parameters and augmented strains of 0.5%, 1.0% and 4.0%. Specimens of 5 inch length were cut from extruded lengths and machined to  $\frac{1}{2}$  inch thickness. Prior to welding, each specimen was degreased and etched to remove oxidation. One specimen of each Alloy 1 to 5 was tested at each strain.

Following the Varestraint test, all specimens were trimmed, ground and polished to reveal weld metal hot

tears on the top surface. These cracks were then evaluated for maximum length and total accumulative crack length.

Results of the tests are presented in Table III, below and FIG. 9. It is believed that the 1% strain data best represents the likely behavior of these Alloys under normal welding conditions. At 1% strain, the alloys can be rated as Alloy 3 having the best performance, Alloy 2 having the worst performance and with Alloys 1, 4 and 5 having intermediate performance to Alloys 3 and 2.

TABLE III

| Alloy | Varestraint (crack lengths in mm) Test Data |      |             |      |             |      |
|-------|---------------------------------------------|------|-------------|------|-------------|------|
|       | 0.5% Strain                                 |      | 1.0% Strain |      | 4.0% Strain |      |
|       | MCL                                         | TCL  | MCL         | TCL  | MCL         | TCL  |
| 1     | 0.06                                        | 0.06 | 1.05        | 5.47 | 2.47        | 22.5 |
| 2     | —                                           | —    | —           | —*   | 4.55        | 28.9 |
| 3     | 0.00                                        | 0.00 | 0.82        | 2.48 | 1.95        | 8.5  |
| 4     | 1.82                                        | —**  | 1.95        | 7.15 | 2.84        | 18.7 |
| 5     | 0.00                                        | 0.00 | 1.83        | 6.13 | 3.36        | 19.2 |

Note:

\*Centerline cracks were observed along the entire length of the weld.

\*\*Bad data point

Varestraint weldability test data is presented in FIG. 10 for alloys 1 to 4, commercial Al-Li alloy 2090, "Weldalite" Al-Li alloy and conventional weldable aluminum alloys 2014 and 2219.

FIG. 10 illustrates the superior weldability performance of Alloys 1 to 4 prepared by the methods of the invention compared to the weldability performance of other weldable Al-Li alloys and conventional aluminum alloys.

Laser weldability evaluations were carried out on Alloy 1 in the as-extruded condition. It was found possible to produce uncracked weld beads with this technique if the laser bursts were programmed for two low power pulses for preheating, one high power pulse for welding followed by two pulses of decreasing power to reduce the cooling rate.

#### EXAMPLE 9

Five 2090 type test alloys (L to P) and seven 8090 type test alloys (E to K) including various amounts of alkali metal impurity were prepared and extruded into flat bar substantially as described above. The concentrations of the principal elements in those alloys in weight percent is presented in Table IV below. In addition, the 2090 alloy of Example 1 (alloy 1) and the 8090 alloy of Example 2 (alloy 2) are listed in Tables IV and V and included in the comparison of mechanical properties.

TABLE IV

| ALLOY | COMPOSITION OF MAJOR ALLOYING ELEMENTS IN AL-LI ALLOYS (WEIGHT PERCENT) |      |      |       |      |       |       |
|-------|-------------------------------------------------------------------------|------|------|-------|------|-------|-------|
|       | Li                                                                      | Cu   | Mg   | Zr    | Sn   | Fe    | Si    |
| E     | 2.02                                                                    | 1.21 | 0.71 | 0.081 |      | 0.05  | 0.031 |
| F     | 2.02                                                                    | 1.21 | 0.71 | 0.082 |      | 0.048 | 0.031 |
| G     | 2.03                                                                    | 1.30 | 0.72 | 0.085 | 0.18 | 0.052 | 0.034 |
| H     | 2.05                                                                    | 1.28 | 0.80 | 0.080 |      | 0.053 | 0.031 |
| I     | 2.01                                                                    | 1.18 | 0.76 | 0.082 |      | 0.048 | 0.029 |
| J     | 1.93                                                                    | 1.15 | 0.71 | 0.110 |      | 0.050 | 0.031 |
| K     | 1.94                                                                    | 1.25 | 0.64 | 0.072 |      | 0.030 | 0.028 |
| L     | 1.95                                                                    | 2.27 | 0.01 | 0.109 |      | 0.051 | 0.028 |
| M     | 2.00                                                                    | 2.45 | 0.01 | 0.101 |      | 0.047 | 0.028 |
| N     | 1.91                                                                    | 2.14 | 0.01 | 0.080 | 0.24 | 0.034 | 0.027 |
| O     | 2.07                                                                    | 2.34 | 0.01 | 0.042 |      | 0.025 | 0.023 |
| P     | 2.04                                                                    | 1.94 | 0.01 | 0.048 |      | 0.049 | 0.025 |
| 1     | 1.96                                                                    | 2.4  | 0.09 | 0.12  | —    | 0.09  | 0.020 |

TABLE IV-continued

| COMPOSITION OF MAJOR ALLOYING ELEMENTS IN AL-LI ALLOYS (WEIGHT PERCENT) |      |      |      |      |    |      |       |
|-------------------------------------------------------------------------|------|------|------|------|----|------|-------|
| ALLOY                                                                   | Li   | Cu   | Mg   | Zr   | Sn | Fe   | Si    |
| 2                                                                       | 1.86 | 1.14 | 0.76 | 0.08 | —  | 0.06 | 0.020 |

The concentration of alkali metal impurities and hydrogen in alloys E to P were determined by GDMS in ppm and are presented in Table V below:

TABLE V

| COMPOSITION OF ALKALI METAL IMPURITIES (GDMS) AND HYDROGEN IN PPM. |       |       |       |        |          |
|--------------------------------------------------------------------|-------|-------|-------|--------|----------|
| ALLOY                                                              | Na    | K     | Rb    | Cs     | H (bulk) |
| E                                                                  | 2.02  | 1.72  | <0.02 | <0.004 | 0.74     |
| F                                                                  | 2.50  | 0.60  |       |        | 0.17     |
| G                                                                  | 4.21  | 0.25  |       |        | 0.27     |
| H                                                                  | 5.3   | 0.58  |       |        | 0.30     |
| I                                                                  | 34.7  | 0.33  |       |        | 0.30     |
| J                                                                  | 12.1  | 0.55  |       | 0.013  | 4.6      |
| K                                                                  | 8.9   | 0.16  |       | 0.004  | 0.25     |
| L                                                                  | 4.6   | 0.2   |       |        | 0.23     |
| M                                                                  | 4.2   | 0.2   |       |        | 6.2      |
| N                                                                  | 1.83  | 0.74  |       |        | 0.2      |
| O                                                                  | 3.4   | 0.74  |       |        | 0.42     |
| P                                                                  | 122   | 39.0  |       |        | 0.33     |
| 1                                                                  | 0.42  | 0.34  |       |        | 0.14     |
| 2                                                                  | 0.54* | 0.20* |       |        | 0.12     |

\*Estimated from the average of 3 similar alloys made at the same time with the same procedure.

Below GDMS detection limits.

The mechanical properties of test alloys E to P, including elongation percent, 0.2% yield strength and Charpy impact values were measured and are plotted in FIGS. 11 to 22. Na+4 K, instead of Na+K, is plotted against mechanical properties in FIGS. 15 to 22 because although Na is the predominant impurity the amount of liquid present in grain boundary regions at room temperature depends strongly on the K concentration because Na is solid at room temperature and the eutectic ratio for Na and K which produces the most liquid for a given weight of impurity and is therefore the most embrittling ratio is about 1 Na : 4 K. In FIGS. 11 to 22 the 0.2% yield strength is plotted against elongation % or Charpy values for alloys 1 and 2 and test alloys E to P grouped according to type.

The data presented in these graphs demonstrates that in each instance increased alkali metal impurities caused a deterioration in 0.2% yield strength, elongation % and Charpy values versus the 2090 and 8090 test alloys.

The plots of yield strength and tensile elongation vs alkali metal impurity in FIGS. 15 to 18 show 2 critical points A and B which are illustrated schematically below.



If the initial composition of an alloy is point C, then a refining process should reduce impurities below point B to be useful. If the initial composition of an alloy is below point B, then any degree of refining will be immediately effective. Increasing degrees of refinement will continue to improve properties until point A is reached at which time the properties will maintain their

high values but no further improvement will occur. Commercial Al-Li alloys are usually in the range A-B. In the case of toughness, the lower critical point has not been reached in any of the alloys made so far. This means that the Na+4 K levels are less than about 1 ppm and the Na+K levels are less than about 0.8 ppm. This suggests that further refinement will continue to improve toughness.

The high plateaus on the yield strength and tensile elongation plots in FIGS. 15 to 18 suggest a region at about 3 ppm Na plus 4 K (e.g., about 1.9 Na plus K) where further reductions in alkali metal impurity has reached a point of diminishing returns for improvement in these properties. However, toughness appears to improve continuously with lower alkali metal impurity levels. For ease of reference alkali metal impurity levels estimated from the data presented in FIGS. 11 to 22, above which degradation of mechanical properties will occur are listed in Table VI below.

TABLE VI

| CRITICAL IMPURITY LEVELS FOR MECHANICAL PROPERTY IMPROVEMENTS IN FLAT BAR EXTRUSIONS |       |                               |                     |                      |
|--------------------------------------------------------------------------------------|-------|-------------------------------|---------------------|----------------------|
| PROPERTY                                                                             | ALLOY | CRITICAL IMPURITY LEVEL (PPM) |                     |                      |
|                                                                                      |       | Na + 4K                       | Na + K at 4:1 ratio | Na + K at 10:1 ratio |
| 0.2% Y.S.                                                                            | 8090  | 5                             | 3.1                 | 3.9                  |
| 0.2% Y.S.                                                                            | 2090  | 3                             | 1.9                 | 2.4                  |
| E1%                                                                                  | 8090  | 3                             | 1.9                 | 2.4                  |
| E1%                                                                                  | 2090  | 3                             | 1.9                 | 2.4                  |
| Charpy                                                                               | 8090  | <1                            | <0.63               | 0.8                  |
| Charpy                                                                               | 2090  | <1                            | <0.63               | 0.8                  |

Unlike tensile strength and elongation %, the impact toughness appears to improve continuously with lower alkali metal impurity levels.

FIG. 23 is a plot of impact toughness calculated in accordance with D. Webster, *Proceedings of the Fifth Al-Li Conference*, Williamsburg, Va., U.S.A. pp. 519-528 (1989), versus alkali metal content (Na+K and Na+4 K) assuming a surface energy reduction mechanism and using the Na plus K grain boundary particles in Al-Li alloys as shown if FIG. 13. The results of this calculated data are similar to the actual data presented in FIGS. 19 to 22.

#### EXAMPLE 10 Aluminum-Magnesium Alloys

Three Al-Mg test alloys A, B and C were prepared to demonstrate the utility of the invention with such alloys by melting commercial 5083 alloy. Alloy A was air melted to simulate commercial practice and contained about 1 ppm Na. Alloy B was vacuum melted and refined to reduce the alkali metal content to below Na levels detectable by emission spectroscopy. Alloy C was melted under argon and doped with Na and K to produce an alloy including about 235 ppm Na. Only the Na content of alloys A, B and C were measured.

Samples of alloys A, B and C were cast in 5 inch diameter molds, extruded to 1 inch round bar at 800° C. and aged at 300° F. for 4 hours. The tensile and impact properties of the aged bars were then tested.

Samples of alloys A, B and C were also cast into 1 inch thick slab ingots and hot rolled at 480° C. to plate and sheet. Samples at various thicknesses were the evaluated for appearance.

FIG. 24 is a plot of the ultimate tensile strength, Charpy impact value, 0.2% yield strength and elonga-

tion % of alloy A, B and C extrusions as a function of Na content. The data presented in FIG. 24 suggests that elongation and toughness are greatest at the lowest Na levels. The changes in yield strength are small. The ultimate tensile strength increases at low Na levels because of the greater ductility of the higher purity alloys.

The rolling behavior of alloy A, B and C slab ingots was evaluated and the results are summarized in Table VII below.

TABLE VII

vacuum was replaced by an argon atmosphere (400 mm Hg) to reduce Mg loss and the melts were cast under argon. The casts were extruded into flat bar. The toughness and tensile properties of the flat bar extrusions and cold rolled sheets were measured and the results are summarized in Table IX below and FIGS. 25 and 26. The toughness and ductility of alloys, X, Y and Z are excellent, but the Na and K levels may be further reduced and the mechanical properties improved by increasing the refining times to further reduce the impurity levels.

TABLE IX

| MECHANICAL PROPERTIES OF MG-LI FLAT BAR EXTRUSIONS IN THE AS EXTRUDED CONDITION |                |                   |           |                 |      |                      |
|---------------------------------------------------------------------------------|----------------|-------------------|-----------|-----------------|------|----------------------|
| Li CONTENT (wt. pct.)                                                           | EXTRUSION SIZE | SPECIMEN POSITION | UTS (ksi) | 0.2% Y.S. (ksi) | EL % | CHARPY VALUE ft. lb. |
| 6.1                                                                             | 3 X 1/2"       | edge              | 36.6      | 24.1            | 16   | 6.1                  |
| "                                                                               | "              | center            | 35.9      | 23.4            | 18   | 5.6                  |
| 14.7                                                                            | "              | edge              | 15.4      | 10.3            | 50   | 51.1<br>not broken   |
| "                                                                               | "              | center            | 15.1      | 10.0            | 40   | 42                   |
| 18.8                                                                            | "              | edge              | 13.3      | 10.2            | 22   | 27.1                 |
| "                                                                               | "              | center            | 13.7      | 10.1            | 27   | 31.3                 |
| "                                                                               | 1 X 0.3"       | edge              | 15.5      | 10.9            | 53   | 34.1                 |
| "                                                                               | "              | center            | 15.5      | 10.9            | 53   | 34.3                 |

THE EFFECT OF IMPURITY LEVEL ON THE HOT ROLLING CHARACTERISTICS OF 5083 PLATE

| ROLLING STEP | ALLOY A<br>(<1 ppm Na) | ALLOY B<br>(<1 ppm Na)    | ALLOY C<br>(235 ppm Na)                             |
|--------------|------------------------|---------------------------|-----------------------------------------------------|
| 23-18 mm     | No cracking            | No cracking               | severe cracking and delamination on the first pass. |
| 18-9 mm      | severe edge cracking*  | no cracking               | rolling discontinued                                |
| 9-6 mm       | severe edge cracking   | very slight edge cracking |                                                     |

\*edges machined to a crack free condition and rolling was continued.

The rolling properties varies significantly with Na concentration. Alloy C slab ingot with 235 ppm Na could not be hot rolled under any conditions without serious cracking and delamination. Alloy A slab ingot could be rolled but not without significant edge cracking. In contrast, vacuum melted alloy B rolled satisfactorily with little edge cracking.

EXAMPLE II Magnesium-Lithium Alloys

Mg-Li alloys X, Y and Z having the compositions set forth in Table VIII below were vacuum refined as described below.

TABLE VIII

| COMPOSITION OF MAGNESIUM - LITHIUM ALLOYS |          |          |          |          |          |        |       |        |        |  |
|-------------------------------------------|----------|----------|----------|----------|----------|--------|-------|--------|--------|--|
| ALLOY                                     | Li Wt. % | Al Wt. % | Mg Wt. % | Fe Wt. % | Si Wt. % | Na ppm | K ppm | Cs ppm | Rb ppm |  |
| X                                         | 6.1      | 3.4      | bal.     | 0.024    | 0.045    | 4.4    | 2.00  | 1.1    | 0.04   |  |
| Y                                         | 14.7     | 0.13     | "        | 0.003    | 0.012    | 7.33   | 5.00  | 1.1    | 0.01   |  |
| Z                                         | 18.8     | 0.17     | "        | 0.008    | 0.098    | 10.0   | 2.50  | 1.4    | 0.01   |  |

Due to the high volatility of Mg these alloys could not be simply melted and vacuum refined. First an initial melt of about 60% wt. Mg and 40% wt. Li was made at about 400° C. and then the melt was further heated to about 500° C. and refined under vacuum for about 20 minutes to reduce alkali metal impurities. Thereafter, the Mg necessary to make the desired alloy composition was added under vacuum and the temperature was raised to 630° C. under vacuum to further reduce the alkali metal impurities. At about 600° C. the

What is claimed is:

1. A process for preparing a high strength aluminum alloy, comprising heating a melt comprised of a base metal of aluminum, greater than 0.5% of lithium, and at least one alkali metal impurity selected from the group consisting of sodium, potassium, rubidium and cesium, to a temperature of about 50° to 200° above the melting point of alloy being refined in a vacuum for a sufficient time to reduce the aggregate concentration of alkali metal impurities in the melt to less than about 5.0 ppm as measured by GDMS.

2. The process of claim 1 wherein the aggregate concentration of alkali metal impurities is reduces to less than about 3 ppm.

3. The process of claim 2 wherein the aggregate concentration of alkali metal impurities is reduces to less than about 0.8 ppm.

4. The process of claim 2 wherein the aggregate concentration of alkali metal impurities is reduces to less than about 0.5 ppm.

5. The process of claim 1 wherein the vacuum is less than about 200  $\mu$ m Hg and the temperature is about 100° C. above the melting point of the alloy being refined.

6. The process of claim 1 wherein the vacuum is less than about 200  $\mu$ m Hg and the temperature is about 50° to about 100° C. above the melting point of the alloy being refined.

7. The process of claim 1, wherein the hydrogen concentration in the melt is reduced to less than about 0.2 ppm, measured by LECO fusion technique.

8. The process of claim 1, wherein the hydrogen concentration in the melt is reduced to less than about 0.1 ppm.

9. A process for making a high strength, high toughness aluminum alloy, comprising the steps of preparing a melt comprised of aluminum and lithium metals including a total of more than 5 ppm of alkali metal impurities selected from the group consisting of sodium, potassium, rubidium and cesium; and reducing the alkali metal impurities so that the total concentration of alkali metal impurities in the alloy is less than about 5.0 ppm.

10. The process of claim 6 further comprising the step of purging the melt with an inert gas.

\* \* \* \*

UNITED STATES PATENT AND TRADEMARK OFFICE  
**CERTIFICATE OF CORRECTION**

PATENT NO. : 5,320,803  
DATED : June 14, 1994  
INVENTOR(S) : Donald WEBSTER

Page 1 of 9

It is certified that error appears in the above-identified patent and that said Letters Patent is hereby corrected as shown below:

In the Drawings

Delete Figures 17-26 and substitute therefor the attached corrected drawings labeled Figures 17-26.

Column 4, line 26, delete "Table II" and insert therefor  
--Table III--.

Column 4, line 28, after "Table III" insert --compared  
with commercially produced aluminum and aluminum-lithium  
alloys--.

UNITED STATES PATENT AND TRADEMARK OFFICE  
**CERTIFICATE OF CORRECTION**

PATENT NO. : 5,320,803  
DATED : June 14, 1994  
INVENTOR(S) : Donald WEBSTER

Page 2 of 9

It is certified that error appears in the above-identified patent and that said Letters Patent is hereby corrected as shown below:

Column 13, line 28 (in Table VII) correct the second column from the left (under the heading "Alloy A") to read (> 1 ppm Na).

Signed and Sealed this  
Twentieth Day of February, 1996

*Attest:*



BRUCE LEHMAN

*Attesting Officer*

Commissioner of Patents and Trademarks



FIG.17



FIG.18



FIG.19



FIG.20



FIG.21



FIG.22



FIG. 23



FIG. 24



FIG.25

